

A. BRIDGE.

METHOD OF AND APPARATUS FOR REDUCING METALS, ETC,  
APPLICATION FILED MAY 29, 1919.

1,415,516.

Patented May 9, 1922.



Inventor

A. Bridge

Watson E. Coleman  
Attorney

# UNITED STATES PATENT OFFICE.

ARTHUR BRIDGE, OF WASHINGTON, DISTRICT OF COLUMBIA.

METHOD OF AND APPARATUS FOR REDUCING METALS, ETC.

1,415,516.

Specification of Letters Patent.

Patented May 9, 1922.

Application filed May 29, 1919. Serial No. 300,587.

To all whom it may concern:

Be it known that I, ARTHUR BRIDGE, a citizen of the United States, residing at Washington, in the District of Columbia, 5 have invented certain new and useful Improvements in Methods of and Apparatus for Reducing Metals, Etc., of which the following is a specification, reference being had to the accompanying drawings.

10 This invention relates to processes for reducing the oxides of metals, such as columbium, molybdenum, tantalum, titanium, tungsten, vanadium and zirconium, and metalloids by means of a thermal reaction 15 with such metals as aluminum, magnesium, and calcium which unite with oxygen to form oxides with great heat of formation.

An object of my invention is to provide a process which will secure pure metals, metalloids and alloys having definite, predetermined proportions of two or more metals or metalloids, and to perform allotropic modifications on elements subject to allotropic changes under high heat and pressure.

25 And a further object is to so control the production of the reaction that there shall be no possibility of explosion which will scatter the materials used.

I attain these objects, broadly speaking, by 30 excluding the oxygen and nitrogen in the air from entering into the reaction by carrying out the reduction process in an entirely closed chamber, and further by using as the means for setting up the thermal reaction an 35 ignition element having the same chemical element as one of the chemical elements entering into the reaction, or by using an extremely small quantity of solid material of different chemical elements than the chemical 40 elements entering into the reaction.

The mechanism whereby the process is carried out is illustrated in the accompanying drawings, wherein:—

45 Figure 1 is a longitudinal section of an apparatus constructed in accordance with my invention;

Figure 2 is a fragmentary view of the igniting wire and its insulation;

50 Figure 3 is a vertical section of another form of apparatus;

Figure 4 is an enlarged fragmentary section of the apparatus;

Figure 5 is a section on the line 5—5 of Figure 4; and

Figure 6 is a section of the apparatus 55 shown in Figure 1 arranged for carrying out a further reaction.

Using one form of mechanism, that illustrated in Figure 1, to carry out my process, I provide a steel cylinder 10, made preferably of seamless, hydraulic steel tubing. Into the ends of this steel cylinder are screwed two heavy steel plugs 11 and 12, thus forming a chamber 13. The plug 11 has a central bore through which is disposed an 60 insulated wire 14. This insulated wire 14 extends through to the interior of the plug 11, the extremity of the insulated wire protruding but a very short distance beyond the inner face of the plug 11. To this end of 65 the insulated wire I attach a wire 15 which is looped and attached by a binding screw 16 or other suitable connection to the inner face of the plug 11. The exterior of the plug is provided with a binding screw 17. 70 Electrical connections may be made to the insulated wire 14 and to the binding screw 17. The loop of wire 15 is of such length that it will extend some distance toward the center of the cylinder when the plug is 75 screwed into position. The wire loop 15 should have, of course, a higher resistance than the wire 14, and this wire may be formed of a metal corresponding to the metal used in reduction, as for instance, aluminum, magnesium, or calcium, and under 80 these circumstances the wire loop is to be insulated with its own oxide or a coating of the oxide to be reduced, or by its own peroxide or a peroxide of the metal to be reduced. In place of such a wire loop as above described, a loop of fine iron wire may be used which is insulated up to a short distance of where it is attached to the insulated 85 wire 14 and binding screw 16 by a layer of tissue paper soaked in a concentrated solution of potassium chlorate, with magnesium powder sprinkled on this insulated layer of tissue paper while it is wet, (see Figure 2) and then dried. The loop of wire of the 90 character before described is designed to serve as an ignition means for starting the thermal reaction, and where an iron wire is used, it may be so small that the chemical elements, iron, carbon, hydrogen, chlorine 95 and potassium, will be found only as minute traces in the final product of the thermal reaction. The loop of wire 15, when coated

with a rather stable oxide, may also be heated by a current below its fusing point to heat the surrounding material for some time before current of greater amperage is applied to fuse the wire. This preheating of the material is, in some cases, of advantage. It will be seen that where a loop of the reducer metal is used, that no other chemical elements are added than the chemical elements entering into the reaction.

After the plug 11 with the ignition device is inserted in the cylinder 10, a heat insulating lining 18 is formed within the cylinder. This lining may consist of such materials as aluminum oxide, magnesium oxide, or calcium oxide. Each of these oxides is a very poor conductor of heat and very refractory. The oxides are used in the form of a calcined powder which is so filled into the cylinder as to provide a central space. The oxide used may correspond to the oxide formed by the thermal reaction, which is of advantage when it is desired to recover as a by-product an unmixed oxide. This central space is to be filled with a reduction mixture 19, that is a mixture of the oxide of the metals or metalloids to be reduced, with one of the reducing metals as aluminum, magnesium, or calcium in a chemically uncombined form. This reduction mixture is in the form of a powder but not necessarily a fine powder except near wire 15, and the constituents of the reduction mixture are mixed in practically the same ratio of proportions by weight as the ratio of their chemical equivalent weights found in a chemical equation representing the reaction. In filling the cylinder, the heat insulating material is packed within the cylinder so as to leave a cavity in the middle into which loop 15 projects. This cavity is filled with the reduction mixture and then a layer of the heat insulating material is packed over it so that the heat insulating material now entirely surrounds the reduction mixture. The plug 12 is next screwed in.

The ignition wire is now connected in an electric circuit and the wire is fused by current of sufficient amperage, whereupon the thermal reaction is started and takes place, this being evidenced by the heating of the cylinder. The cylinder and contents are allowed to cool before the contents are taken out and separated.

Where the process is to be carried out on a relatively extensive scale, the apparatus shown in Figure 3 would be preferably used. In this case, 20 designates a metallic form or holder having therein connected chambers 21 and 22, the chamber 21 being smaller in diameter than the chamber 22, and there being an opening 23 communicating with the chamber 22 adjacent its junction with the chamber 21. Disposed within the cham-

ber 22 is a piston 24 having a length longer than the size of the opening 23, the chamber 22, however, being of sufficient length so that the piston 24 can move back into the outer end of the chamber 22 to disclose the opening 23. Disposed within the chamber 21 is a piston 25, and the chambers 21 and 22 are connected by ducts 26 to means whereby fluid under high pressure, as for instance, water may be forced into these chambers to thereby force these pistons 24 and 25 towards each other. The thermal reaction is carried out within a metallic case 29 having a loose cover 30, which is adapted to fit within the chamber 21 and which contains an outer layer of heat insulating material 18 surrounding a central mass 19 of the reducing mixture. The ignition means in this instance consists of a loop of wire 15<sup>a</sup> connected to double leads 14<sup>a</sup> which extend out through the top or cover 30 and extended laterally in a groove therein, which groove is filled with cement after the crucible lid is set on the crucible 29, the wires being carried out through the opening 23. Of course, I do not wish to be limited to this, as other means of ignition might be provided.

With an apparatus of this character, the thermal reaction is precisely the same as in the apparatus previously described, but instead of having a very heavy cylinder of relatively small capacity, I dispose the reducing mixture within a relatively light case 29 and dispose this in a holder which is relatively strong so that the pressure within the case will not act to burst it. In this construction, the case or crucible, as it may be termed, is inserted through the opening 23, and disposed in the upper end of the chamber 21. Then fluid is admitted beyond the piston 24 to force the case 29 inward into the chamber 21, and when the piston 24 has fully seated and fully closes the opening 23, then the piston 25 is urged upward until it seats against the case 29. Thus, the case is entirely surrounded by heavy metallic walls which will resist the pressure generated within the case and prevent the case from being ruptured. After a certain lapse of time, during which the reaction is completed, the pressure of the confined gases is relaxed by relieving the hydraulic pressure behind the piston 24 a little. The pressure within the container or crucible 18 will then raise the lid 30 a trifle, permitting the gases to escape through the opening 23. After this, the hydraulic pressure is applied behind the piston 25 and relieved from behind the piston 24 to cause the upward movement of the pistons 25 and 24 to carry the case 29 and its contents into position in front of the opening 23 and permit the removal of the case by tongs.

While I have heretofore described the

lining of the crucible by simply packing a powdered heat insulating material around the wall of the crucible, a more or less permanent lining of magnesium oxide to the 5 wall of the crucible may be formed by fitting the metal shell of the crucible, illustrated in Figure 1, or the metal shell of the container 29, with a temporary water jacket connected by flexible hose to a source of 10 water. The magnesium oxide may be applied by means of an electric arc brought into contact with unfused magnesium oxide placed within the cylinder. This melts the magnesium oxide near the arc and causes it 15 to adhere to the water cooled metal crucible. Small quantities of magnesium oxide are added as needed and the arc shifted, and thus a complete interior lining may be built up within the crucible, this lining 20 being applied by the means above described to the head or end of the crucible.

It will be seen that with the construction described, I reduce metals, metalloids and alloys without the oxygen and nitrogen of the 25 air entering into the chemical reaction at all. This is particularly essential in the case of refractory acid forming metals which will not readily fuse into a regulus, and in some cases will not fuse into a regulus at all, and 30 as they combine with oxygen and nitrogen while at a high temperature, they cannot be reduced in the air by a thermal reaction without causing a secondary reaction with the oxygen and nitrogen of the air directly 35 after being reduced. This secondary reaction is always more or less complete according to the physical condition and chemical nature of the metal reduced.

It will be noted that there is no secondary 40 reaction where my process and apparatus is used. Furthermore, my process is advantageous in that as the space in which the reaction takes place is entirely enclosed, there can be no volatilization of the metal acting 45 as the reducing agent or the metal oxide being reduced. Furthermore, by having this process take place in an entirely closed chamber, there is no scattering of the material used in the reduction and no heat is lost 50 by the unrestricted expansion of the volatile material, and there is no possibility of explosions occurring which would scatter or displace the material being treated. Heretofore, the reduction of such metals as columbium, molybdenum, etc., have been secured by means of carbon reduction in an electric arc furnace. This produces brittle 55 metals with a carbon content in the cases of these metals as columbium, tantalum, vanadium, zirconium, molybdenum and others. Carbon free metal has been produced by pulverizing the reduced metal, mixing it with sufficient metallic oxide to react with the carbon, and the reduction effected by insertion 60 in a crucible in an arc furnace, but my 65

method has an advantage over the one just described, in that there is only one operation instead of two, and further the secondary reactions with air are entirely eliminated.

The method heretofore described and an 70 apparatus, similar to that illustrated in Figure 1, is also adapted for the purpose of producing an allotropic form of carbon, in other words producing a diamond. In Figure 6, I show the same form of cylinder as is illustrated in Figure 1. I use a reduction mixture 32 which is composed of magnesium carbonate and metallic magnesium ( $MgCO_3 + Mg$ ). An insulating lining 33 of fused or powdered magnesium oxide is 80 also used between the mass of the reduction mixture 32 and the walls of the crucible. Disposed in the lower portion of the mass of reduction mixture is a lump 34 of pure 85 carbon, as for instance, in the form of graphite, and disposed within the mass of the reduction mixture is a container 35 of magnesium which is filled with some inert gas under compression, as for instance, a gas of the helium series, such as argon. 90

It will be seen that the process just above described is but a carrying forward of the process previously described, in that the same process of thermal reaction is used but the heat and pressure produced by this reaction is used to change the form of an allotropic element. The purpose of the container 35 with its compressed helium gas is to cause the pressure to be maintained within the chamber until the critical temperature 95 necessary for the production of a diamond has passed, the expansion of the gas after the reduction has been secured maintaining this pressure. Without this container and 100 gas, the necessary pressure would not be 105 maintained. It will be seen that this process is similar to the process of metal reduction heretofore described, in that the magnesium carbonate corresponds to the metallic oxide. It differs from the previous process, however, merely in the fact in the use of the small gas container and the disposal within the chamber of a lump of graphite to be 110 acted on by the heat and pressure.

In the reaction of the magnesium-magnesium carbonate mixture, the magnesium carbonate is not decomposed into the components  $Mg + C + 3O$  having 266.6 calories but the magnesium remains combined with its equivalent oxygen, the components being  $MgO + C + 2O$ . This takes 143.3 cal., the heat of formation of  $Mg + O$  from 266.6 cal., which gives 123.3 cal., then the heat represented by the reaction of  $2Mg$  on  $MgCO_3$  would be  $143.3 \times 2 - 123.3$ , which gives 163.3 125 cal., an exothermic reaction in which great heat is developed.

Graphite, in common with other materials, increases greatly in compressibility by the application of heat and under the reaction 130

used by my method great heat is developed. As before stated, the reaction secures 163.3 calories of heat and this amount of heat applied to 133 grams of material having approximately an average specific heat of .3 will give a temperature of nearly  $4000^{\circ}$  C. above the temperature before reaction. With a small piece of graphite heated above  $3000^{\circ}$  C. a very great pressure is not believed to be necessary in order to convert it into a diamond and if the inert gas was heated to, say  $2730^{\circ}$  above its original temperature and would expand to twice its volume after release, it would exert five times the pressure it was originally under in the container and this original pressure may easily be 200 atmospheres. It is believed, therefore, that ample pressure would be secured to secure the allotropic modification under the reaction described.

Another method of carrying out an allotropic modification on elements subject to allotropic changes under high heat and pressure is to use such a construction as that illustrated in Figures 1 or 6, but in place of using a container 35 holding inert gas, I would simply use with the reduction mixture, composed of the oxide of the metals or metalloids to be reduced, with one of the reducing metals, as aluminum, magnesium or calcium in a chemically uncombined form, an excess of magnesium, in case magnesium is used, which forms a metallic vapor or liquid when the reaction takes place, thus securing the desired pressure within the cylinder, which pressure is maintained within the cylinder or chamber until the critical temperature necessary for the production of a diamond has passed by the vaporization of the excess magnesium after the reduction has been secured. The wire 15 in this case should be relatively long and preferably of magnesium coated with magnesium oxide. The contents of the crucible should be preheated by wire 15 before the reaction is started. This process differs from that previously described with reference to Figure 6, merely in the fact that in this last case I use an excess of magnesium and preheat the contents of the chamber.

In Figures 1 and 6 I have illustrated the plugs 11 and 12 as being formed with air vents which are opened when the plugs are inserted to permit the outward passage of air and which are then closed by plugs 36.

I claim:—

1. A method of reduction which consists in disposing within a closed, air-tight, pressure resisting chamber a mass of mixed materials of such a nature that they will undergo thermal reaction upon initial ignition, insulating said mass from the walls of the chamber, and causing an initial ignition of the mass to thereby effect reduction.

2. A method of reduction which consists in disposing within a closed, air-tight, pressure resisting chamber a mass of mixed materials of such a nature that they will undergo a thermal reaction upon an initial ignition, insulating said mass from the walls of the chamber, causing an initial ignition of the mass, releasing the pressure of gas within the chamber after the reduction is completed, and removing the reduced material from the chamber.

3. A method of reducing the oxides of metals and metalloids which consists in disposing within a closed, air-tight and pressure resisting chamber a mixture of oxides of the material to be reduced with a metal which unites with oxygen to form oxides with high heat of formation, insulating the mixture thus formed from the wall of the chamber, and initially igniting the material to start the reaction.

4. A method of reducing the oxides of metals, metalloids and alloys, which consists in disposing within a closed, air-tight and pressure resisting chamber a mixture of the oxide of the metal to be reduced together with a metal which will unite with oxygen to form an oxide with high heat of formation, and insulating the reducing mixture so formed from the walls of the chamber by a layer of an oxide of a metal corresponding to the oxide to be formed by the thermal reaction, and initially starting the reaction by igniting the mixture.

5. A method of reducing the oxides of refractory acid forming metals such as columbium, molybdenum, tantalum, titanium, tungsten, vanadium, etc., by means of a thermal reaction with such metals as aluminum, magnesium, and calcium, which consists in lining a closed, air-tight and pressure resisting chamber with a layer of heat insulating material composed of the particular oxide to be formed by the thermal reaction, said material being in the form of a calcined powder, then filling the space enclosed by the heat insulating material with a mixture of the oxide of one of the refractory acid forming metals with one of the reducing metals in a chemically uncombined form, the mixture being in the form of a powder and being mixed in approximately the same ratio of proportions by weight as the ratio of their chemical equivalent weights found in a chemical equation representing the reaction, and then applying heat to said mixture to cause an initial reaction.

6. A method of reducing the oxides of metals and metalloids, which consists in lining a closed, air-tight and pressure resisting chamber with a heat insulating lining composed of the particular oxide corresponding to the oxide to be formed by the thermal reaction, disposing within the space

enclosed by said lining a reduction mixture comprising the oxide of metals to be reduced with one of the reducing metals in a chemically uncombined form, and initially igniting said reduction mixture to cause thermal reaction to start.

7. A method of producing an allotropic modification of a mineral body by subjecting it simultaneously to high pressure and 10 a temperature sufficiently high to secure such modification, which consists in disposing within a closed, air-tight and pressure resisting chamber lined with insulating material, a reduction mixture comprising an 15 oxide of a metal or metalloid with a reducing metal in a chemically uncombined state, disposing within said mass of reduction mixture a lump of the mineral to be modified, and disposing within the mass of reduction mixture a fusible body which, when subjected to a high temperature, will liberate a gaseous elastic vapor, and heating and 20 igniting the reduction mixture to start thermal reaction within said chamber to thereby produce a high temperature and 25 simultaneously fuse the said body to secure and maintain an extremely high pressure within the chamber while the modification is being effected.

30 8. An apparatus for the purpose de-

scribed comprising a chamber having relatively heavy walls, and having a filling opening and means for closing said opening, one wall of the chamber having extending through it an insulated wire, and a loop of 35 electrically fusible metal connected to said wire and extending into the interior of the chamber.

9. A mechanism of the character described comprising a hollow body having relatively thick walls and formed to provide two connected chambers having different diameters, one chamber opening directly into the other, pistons, one in each chamber, means for applying pressure to 40 said pistons to force them towards each other, the wall of the larger chamber having an opening normally closed by the piston of the larger chamber when it is forced fully in one direction but disclosed by said 45 piston when it is forced fully in the other direction into the space between said pistons, and including an electrically fusible, metallic loop.

In testimony whereof I hereunto affix my 55 signature in the presence of two witnesses.

ARTHUR BRIDGE.

Witnesses:

FREDERIC R. WRIGHT,  
ROBERT A. BOSWELL.